

Patented Dec. 7, 1948

2,455,427

# UNITED STATES PATENT OFFICE

2,455,427

## PROCESS FOR IMPREGNATING WOOD AND COMPOSITION THEREFOR

William Karl Loughborough, Madison, Wis., assignor to United States of America as represented by the Secretary of Agriculture

No Drawing. Application March 9, 1945,  
Serial No. 581,821

6 Claims. (Cl. 117—148)

(Granted under the Act of March 3, 1883, as amended April 30, 1928; 370 O. G. 757)

1

This application is made under the act of March 3, 1883, as amended by the act of April 30, 1928, and the invention herein described and claimed, if patented, may be manufactured and used by or for the Government of the United States of America for governmental purposes without the payment to me of any royalty thereon.

This is a continuation-in-part of my copending application, Serial No. 462,191, filed October 15, 1942, now Patent No. 2,442,897, which, in turn, is a division of my application, Serial No. 383,798, filed March 17, 1941, upon which Patent No. 2,313,953, issued on March 16, 1943.

This invention relates to the chemical seasoning of wood and particularly to the use of water-soluble, diffusible resin-forming chemicals in the chemical seasoning process.

The principal object of my invention is to provide a chemical seasoning process that will eliminate or minimize seasoning defects during the drying of refractory items of wood, such as occurs with ordinary drying or chemical seasoning methods.

Other objects of my invention are to permit, for various woods, faster drying than can be obtained with ordinary drying or chemical seasoning methods or to permit less exacting control of humidity conditions than is required in other seasoning processes. Further objects are to provide a chemical seasoning agent that does not corrode metal equipment used in the drying process or metal devices which might be used with the dried wood, which will not materially injure the inherent electrical properties of the wood, which does not discolor wood, and which protects the wood during seasoning, and, to a certain extent, during use subsequent to drying, against fungal stain, decay, insect damage, and fire.

Still further objects of my invention are to provide a chemical seasoning process which will yield a product that is non-hygroscopic and which has permanent antishrink properties and increased strength across the grain.

The first step in the process of chemical seasoning is the deposition within the outer layers of water-swollen wood of one or more hygroscopic and antishrink chemical agents. The expressions "outer layers" and "outer zone" as used hereinafter refer to that portion of the wood be-

tween the surface and a depth of about  $\frac{1}{5}$  the distance from the wide surfaces to the plane midway between the wide surfaces.

The first step is usually accomplished by soaking the green wood in a comparatively concentrated solution of the chemical agent. Although the water vapor pressure of such a solution is considerably lower than that of the water in the wood, and some is removed from the wood during the soaking, the wood is usually taken from the solution before much drying has occurred, and most of the drying is accomplished by exposing the wood to a drying atmosphere.

When the chemical agents are absorbed, the relative vapor pressure of the water in the treated portion of the wood is lowered, and such portion is given water retention properties not possessed by untreated wood. The process reverses the normal stresses that develop in wood as it dries by causing the wood in the outer layers to retain moisture above its fiber saturation point, and thus it remains in a turgid condition even though a normal drying gradient is set up in the interior of the wood. The chemical agent also diffuses into the cell walls of the wood where it prevents the wood from shrinking as much as it would if no chemical were present.

Heretofore, simple organic or inorganic compounds, such as sodium chloride, monoammonium phosphate, urea, diethylene glycol, glycerine, invert sugar or mixtures of such compounds have been employed in chemical seasoning processes. However, many of them, such as urea, do not have adequate hygroscopic and antishrink effect during the drying period adequately to decrease checking and honeycombing of thick pieces of refractory woods, such as oak. Those that are most effective for reducing degradation of refractory woods have other disadvantages. For example, sodium chloride is so corrosive that it cannot be used in a kiln containing any ferrous metal fixtures, and the presence of the ionizable salt in the dried wood lowers its electrical resistance. Diethylene glycol, glycerine, and similar compounds are too expensive for general use. Urea alone or in combination with chemicals such as invert sugar, corn sugar, or molasses discolor wood. Compounds that tend to maintain their hygroscopic properties after the wood has been dried result in the treated wood having a

tendency to absorb more moisture than untreated wood when exposed to high relative humidities and to condense moisture on its surface when exposed, even for short periods, to very high relative humidities. Furthermore, chemical seasoning agents of the prior art require a high degree of precision in the control of kiln conditions. For example, when the humidity becomes appreciably higher than the relative humidity in equilibrium with a saturated solution of chemical seasoning agents of the prior art, excessive moisture is absorbed by and condenses on the wood. If exposure to this humidity is prolonged, the water will drip from the lumber, leaching out the protective chemical agent. On the other hand, if the relative humidity becomes appreciably lower than the relative humidity in equilibrium with a saturated solution of the chemical seasoning agent, the agent will not be effective in maintaining sufficient moisture in the wood to prevent checking, especially if excessive humidity at some previous time has leached out part of the chemical.

My invention obviates to a large extent the deficiencies of the prior art pointed out above by utilizing essentially monomeric water-soluble resin-forming compounds in the chemical seasoning process. The essential attributes of such compounds that are effective in carrying out the objects and purposes of my invention are that their molecules have comparatively small size and a structure such as to permit their ready diffusion into the free and hygroscopic moisture of the wood. Also, these compounds are sufficiently effective in lowering the relative vapor pressure of the water in the wood, and they eventually polymerize in the fine swelling structure of the wood during the latter stages of the drying process, forming a resin that has no appreciable hygroscopic properties.

Buffers or other modifying agents may be used to assist in maintaining the resin-forming compounds in a diffusible state and in regulating the formation of the non-hygroscopic resin during the latter stages of the drying. Special heating or conditioning periods or secondary chemical treatments at the end of the drying may also be employed to complete the setting of the resin if required in any particular case. Other chemical agents may be added to the treating solution to obtain increased protection against stain, decay, insects, and fire.

Buffered urea-aldehyde solutions, described in Patent No. 2,313,953 and in my copending patent application, Serial No. 462,191, filed October 15, 1942, are especially useful in the practice of my present invention.

It is essential that the chemical agent be confined largely to the outer layers of the wood. For this purpose, I have found it satisfactory to soak the unseasoned wood in an aqueous solution of the chemical agent 3 to 4 days per each inch of thickness of the wood.

In order for the chemical seasoning agent to accomplish its purpose, its concentration in the outer layers of the wood must be high, and accordingly the concentration of the chemicals in the treating solution must be high. Solutions in which the combined weights of the urea and formaldehyde components make up 40 to 60 percent of the total weight are preferred for this purpose.

Dimethylolurea may be substituted for the formaldehyde and a portion of the urea in preparing the buffered urea-aldehyde solution. Also,

thiourea may be used as a substitute for or in admixture with urea in the buffered urea-aldehyde solution. Other aldehydes, such as acetaldehyde, may also be used in the solution.

5 Examples of typical solution formulae which have been successfully used in the chemical seasoning of oak in accordance with my invention are:

## FORMULA I

|                                       | Grams |
|---------------------------------------|-------|
| Water                                 | 231   |
| Sodium hydroxide                      | 6     |
| Borax                                 | 39    |
| Urea                                  | 380   |
| 15 Formaldehyde (37 percent solution) | 344   |
|                                       | 1000  |

## FORMULA II

|                                                       | Grams |
|-------------------------------------------------------|-------|
| Water                                                 | 416   |
| Sodium hydroxide                                      | 6     |
| Borax                                                 | 39    |
| 25 Dimethylolurea (89 percent pure, 11 percent water) | 286   |
| Urea                                                  | 253   |
|                                                       | 1000  |

30 Although the formulae given above, which produce solutions having, approximately, pH 10, are suitable for use with oak, which is a highly acid wood, other woods that are not so highly acid may require the omission of the sodium hydroxide or the addition of glacial acetic acid to reduce the pH of the solutions to the approximate range of 8 to 9. I have found such a pH to be ideally suited for maintaining the resin-forming compounds in a virtually unpolymerized state so that the treating solution is available for a longer period of time and, more importantly, the compounds are maintained in a diffusible state without losing their hygroscopic properties during the early stages of the drying.

45 The buffered urea-aldehyde solutions described above tend to bleach the wood rather than to darken it as in the case of urea or urea in combination with compounds such as diethylene glycol, invert sugar, and molasses. The urea-aldehyde resin present in the wood after drying does not lower the electrical resistance of the wood as do inorganic salts. After completion of the drying, the urea-aldehyde resin is non-hygroscopic.

50 55 Wood which has been dried with the aid of the resin-forming compounds is less hygroscopic than untreated wood and much less hygroscopic than wood treated with simple hygroscopic chemical agents heretofore used in the chemical seasoning process. It absorbs less moisture from air which has a high relative humidity than untreated wood, and much less moisture than, for example, wood treated with urea. Moisture does not condense upon the surface of the resin-treated wood

60 65 when it is exposed to very high humidities. The urea-formaldehyde resin cannot be leached out of the wood after drying is completed. Thus, the antishrink effect which is obtained by the treatment of the wood with the buffered urea-aldehyde solution is permanent. The urea-formaldehyde treated wood is not affected by stain or decay fungi when exposed to high humidities during or after drying. The treatment also increases the fire resistance of the wood.

70 75 Using a buffered urea-aldehyde solution, a

satisfactory procedure comprises preliminary soaking of the unseasoned wood in the solution for about 3 or 4 days per inch of thickness of the stock. The wood is then dried in a drying chamber under controlled temperature conditions with humidity conditions maintained in the beginning at approximately the relative vapor pressure of air in equilibrium with the treating solution. The drying conditions are then adjusted so as finally to dry the wood to the desired moisture content, which will usually be about 3 to 15 percent by weight but may be as high as 30 percent or higher.

Another procedure which may be employed comprises preliminary soaking of the unseasoned wood in a buffered urea-aldehyde solution, the soaking period being about 3 or 4 days per inch of thickness of the stock, and then either drying the wood under air-drying conditions until it is dried to the desired moisture content or partially drying it under such conditions and then completing the drying in a drying chamber under controlled conditions.

Although most satisfactory results are obtained when the chemical agent is applied by the soaking method, other means of application may also be used in the practice of my invention. For example, I have found it suitable to apply the solution in the form of a paste to the surface of the wood followed by piling the wood so as to cause the resin-forming compounds to diffuse into the wood. This may be accomplished by piling the paste-treated wood solid, or on very thin stickers, preferably under a waterproof cover, and leaving it so piled until the chemical agents have diffused into the wood. Stickers about  $\frac{1}{8}$  inch thick are satisfactory in using this method. The diffusion period is about the same as required in the soaking method. After the diffusion period, the treated wood is dried in the same manner as the soaked wood.

Another means of handling such paste-treated wood is to pile the wood on stickers within a drying chamber, then maintain the relative humidity of the air in the chamber at equilibrium with the relative vapor pressure of the chemical seasoning agent until the chemical compounds have diffused into the wood. The drying phase is then effected.

In carrying out the variations described above, any thickening agent which will increase the viscosity of the treating solution without adversely affecting its properties or the properties of the wood being treated can be used, such as cornstarch, methylcellulose, bentonite, and methylcellulose in combination with bentonite. Any other hydrophilic thickening agent may be used. The paste can be applied by dipping, brushing, spraying, or other means. The amount of chemical seasoning agent retained by the water-swollen wood when the paste is applied by dipping, brushing, spraying, and so forth, may be controlled by varying the amount of thickening agent used and by other means, such as regulation of temperature, and so forth. The amount of chemical seasoning agent required will depend upon the size and kind of wood being dried, but the practical range is from about 40 to about 200 pounds of resin-forming compounds per thousand board feet of wood.

Under some circumstances, and for some wood pieces, it may be satisfactory to impregnate the outer zones of the unseasoned wood with the treating chemicals by means of a pressure or vacuum-pressure treatment.

The following examples illustrate my invention

5 in more detail and the manner in which it may be practiced:

EXAMPLE 1

*Soaking and kiln drying method*

6 Forty pieces of unseasoned white oak heartwood 4 by 6 inches in cross-sectional dimension and 30 inches in length, which had been selected at random from a large group of such pieces, were soaked for 12 days in a buffered urea-aldehyde solution containing the following ingredients:

|                                    | Parts by weight |
|------------------------------------|-----------------|
| Water                              | 231             |
| Sodium hydroxide                   | 15 6            |
| Borax                              | 39              |
| Urea                               | 380             |
| Formaldehyde (37 percent solution) | 344             |
|                                    | 1000            |

20 The first four ingredients listed were mixed together in the order shown while heating to 150° F. The last ingredient was added after the mixture was cooled to approximately 100° F. The temperature of the solution during soaking was about 80° F.

25 After the soaking period, the ends of the pieces were treated with a moisture-resistant coating to prevent moisture loss from the ends of the pieces and consequent end checking. The soaked and end-coated pieces were piled on 1-inch stickers in a drying chamber along with 40 similar end-coated pieces which had been soaked 12 days in a saturated urea solution at approximately 80° F. and 35 40 similar end-coated pieces which had not been given any chemical seasoning treatment. All these pieces were then dried to a moisture content of approximately 12 percent, based on the oven-dry weight of the wood, using the following drying schedule:

| Elapsed time, days | Temperature   |               | Relative humidity, percent | Moisture content of untreated specimens, percent |
|--------------------|---------------|---------------|----------------------------|--------------------------------------------------|
|                    | Dry bulb, °F. | Wet bulb, °F. |                            |                                                  |
| 0                  | 115           | 111           | 88                         | 88.0                                             |
| 32                 | 117           | 112.5         | 87                         | 47.0                                             |
| 40                 | 115           | 111           | 88                         | 44.0                                             |
| 51                 | 115           | 108           | 79                         | 35.5                                             |
| 90                 | 115           | 105           | 71                         | 32.4                                             |
| 111                | 115           | 102           | 64                         | 25.7                                             |
| 130                | 115           | 93            | 44                         | 21.0                                             |
| 146                | 135           | 109           | 43                         | 17.0                                             |
| 174                |               |               |                            | 12.0                                             |

55 The following table shows the influence of the buffered urea-aldehyde treatment:

TABLE A

| Treatment                      | Total length in inches   |                                      |
|--------------------------------|--------------------------|--------------------------------------|
|                                | Surface checks per piece | Honeycomb checking per cross-section |
| Buffered urea-aldehyde, soaked | 49.6                     | 1.15                                 |
| Urea, soaked                   | 80.0                     | .97                                  |
| None                           | 153.4                    | 2.80                                 |

60 When drying was completed, the urea-treated oak was considerably darkened compared with the untreated controls, but the buffered urea-aldehyde treated wood was not darkened. At high humidities, the urea-treated and dried stock absorbed more moisture from the air than the buffered urea-aldehyde treated and dried stock.

At humidities above 85 percent, the urea-treated stock condensed moisture on its surface, whereas the buffered urea-aldehyde treated stock did not condense moisture on its surface even at humidities up to 100 percent.

## EXAMPLE 2

## Paste-piling and kiln drying method

Forty pieces of unseasoned white oak heart-wood 4 by 6 inches in cross-sectional dimensions and 30 inches in length, which had been selected at random from a large group of such pieces, were

piled on  $\frac{1}{8}$  inch thick stickers 15

covered for 12 days after having been surface coated with a paste consisting of the following ingredients:

|                                                    | Parts by weight |
|----------------------------------------------------|-----------------|
| Water                                              | 38.50           |
| Sodium hydroxide                                   | .56             |
| Borax                                              | 3.59            |
| Dimethylolurea (87 percent pure, 11 percent water) | 26.50           |
| Methylcellulose                                    | 3.70            |
| Urea                                               | 23.40           |
| Bentonite                                          | 3.75            |

The sodium hydroxide, borax, and dimethylolurea were dissolved in two-thirds of the water while heating to 150° F., and the solution was cooled to 80° F. The methylcellulose was wetted in the rest of the water at 180° F., and this mixture was cooled to 80° F. The urea and the solution were then added simultaneously to the methylcellulose-water mixture while stirring. The bentonite was then added to the entire mixture while stirring. The paste was applied at the rate of 150 pounds of solid chemical per thousand board feet of the wood. After the diffusion period, the ends of the pieces were treated with a moisture-resistant coating to prevent moisture loss from the ends and consequent end checking. The treated and end-coated pieces were piled on 1-inch stickers in a drying chamber along with 40 similar end-coated pieces which had been treated 12 days with an urea-methylcellulose paste and 40 similar end-coated pieces which had not been given any chemical seasoning treatment. The urea paste was applied at the rate of 150 pounds of urea per thousand board feet, and the stickering and covering conditions were the same as for the buffered urea-aldehyde paste-treated wood during the diffusion period.

All the pieces were then dried to a moisture content of approximately 12 percent using the drying schedule given in Example 1. The following table shows the influence of the buffered urea-aldehyde treatment.

TABLE B

| Treatment                           | Total length in inches   |                                      |
|-------------------------------------|--------------------------|--------------------------------------|
|                                     | Surface checks per piece | Honeycomb checking per cross-section |
| Buffered urea-aldehyde, paste-piled | 54.3                     | 1.47                                 |
| Urea, paste-piled                   | 138.3                    | 2.55                                 |
| None                                | 153.4                    | 2.80                                 |

When drying was completed, the color and hygroscopic properties of the buffered urea-aldehyde paste and urea paste-treated pieces were similar to those of the corresponding pieces treated by those two chemical seasoning agents by the

## EXAMPLE 3

## Soaking and air seasoning method

Twenty pieces of unseasoned white oak heart-wood 3 by 6 inches in cross-sectional dimensions and 30 inches in length which had been selected at random from a large group of such pieces were soaked for 20 days in a buffered urea-aldehyde solution prepared as described in Example 1. After the soaking, the ends of the pieces were coated with a moisture-resistant material to prevent moisture loss from the ends of the pieces and consequent end checking. The soaked and

the open air along with 20 similar end-coated pieces which had been soaked 20 days in a saturated urea solution and 20 similar end-coated pieces which had not been given any chemical seasoning treatment. All these pieces were allowed to dry to a moisture content of 20 to 25 percent under the uncontrolled conditions of air drying. When the air drying was completed, the pieces were further dried to 12 percent moisture content in a drying chamber under controlled temperature and humidity conditions. The following table shows the influence of the buffered urea-aldehyde treatment:

TABLE C

| Treatment                      | Total length in inches   |                                                        |
|--------------------------------|--------------------------|--------------------------------------------------------|
|                                | Surface checks per piece | Honeycomb checking per cross-section after kiln drying |
| Buffered urea-aldehyde, soaked | 61.4                     | 0.64                                                   |
| Urea, soaked                   | 140.5                    | 3.91                                                   |
| None                           | 138.0                    | 1.42                                                   |

When drying was completed, the color and hygroscopic properties of the buffered urea-aldehyde urea-treated pieces were similar to those of the corresponding pieces treated by those two chemical seasoning agents and kiln dried.

## EXAMPLE 4

## Drying under more severe schedules and less exact temperature and humidity control than permissible with ordinary drying methods

Ten unseasoned sugar maple sapwood shoe last blanks, size No. 11, were soaked for 5 days in a buffered urea-aldehyde solution of the composition shown in Example 1. After the soaking period, the ends of the blanks were coated with a moisture-resistant material to prevent moisture loss from the ends and consequent end checking. The soaked and end-coated pieces were piled on 1-inch stickers in a drying chamber and dried to a moisture content of approximately 5 percent using the following drying schedule:

| Elapsed time, Days | Temperature   |               | Relative humidity, Percent | Estimated moisture content, Percent |
|--------------------|---------------|---------------|----------------------------|-------------------------------------|
|                    | Dry bulb, °F. | Wet bulb, °F. |                            |                                     |
| 0                  | 140           | 120           | 54                         | 63.4                                |
| 7                  | 160           | 140           | 59                         |                                     |
| 17                 | 160           | 125           | 37                         |                                     |
| 21                 | 170           | 135           | 39                         |                                     |
| 25                 | 170           | 127           | 30                         |                                     |
| 30                 | 180           | 137           | 32                         |                                     |
| 36                 |               |               |                            | 5.0                                 |

The blanks dried without defect, were non-hygroscopic, and were darkened only slightly compared

with untreated blocks dried under considerably milder conditions. Unseasoned maple shoe last blanks which have not been chemically treated cannot ordinarily be dried without defect under such severe initial temperature and humidity conditions. Ordinary commercial kiln drying facilities are not capable of drying unseasoned shoe last blanks without chemical treatments in less than 60 days.

Although it is not possible at present to state with certainty what phenomena are responsible for the high effectiveness of the buffered urea-aldehyde solutions in the chemical seasoning process, it is known that the chemicals when impregnated into the wood possess both the hygroscopic and antishrink properties desirable for the process. In the resinified form the absorbed urea-aldehyde improves the bond between adjacent and contiguous fibers, thereby increasing the strength of the wood in tension across the grain. This property probably is of some assistance in preventing the formation or enlargement of wood failures which appear as checks.

Having thus described my invention, I claim:

1. A process for seasoning refractory wood comprising soaking the wood in an aqueous solution containing urea and formaldehyde in the relative molal proportions of about 6 to 4, respectively, said solution being buffered to a pH in the range of about pH 8 to about pH 10.5, followed by drying the treated wood.

2. A process for seasoning refractory wood comprising soaking the wood in an aqueous solution containing urea and formaldehyde in the relative molal proportions of about 6 to 4, said solution being buffered to a pH in the range of about pH 8 to about pH 10.5, followed by drying the wood to a moisture content of about 3 to 15 percent, by weight.

3. A process for seasoning refractory wood comprising applying urea-formaldehyde resin-forming compounds to the surface of the wood at the rate of about 40 to 200 pounds per thousand board feet, the compounds being applied in the form of a solution buffered to a pH in the range of about pH 8 to pH 10.5 and thickened with a hydrophilic thickening agent, the urea and form-

aldehyde being present in the relative molal proportions of about 6 to 4, permitting the resin-forming compounds to diffuse into the wood, followed by drying the treated wood.

5. As a composition for the chemical seasoning of wood an aqueous solution of 40 to 60 percent by weight of a mixture of urea and formaldehyde in the relative molal proportions of substantially 6 to 4, respectively, said solution being buffered to a pH in the range of substantially pH 8 to 10.5.

15. As a composition for the chemical seasoning of wood an aqueous solution of 40 to 60 percent by weight of a mixture of urea and formaldehyde in the relative molal proportions of substantially 6 to 4, respectively, said solution being buffered to a pH in the range of substantially pH 8 to 10.5 and containing a hydrophilic thickening agent.

20. As a composition for the chemical seasoning of wood an aqueous solution of 40 to 60 percent by weight of a mixture of urea and formaldehyde in the relative molal proportions of substantially 6 to 4, respectively, said solution being buffered to a pH in the range of substantially pH 8 to 10.5 and containing starch.

WILLIAM KARL LOUGHBOROUGH.

#### REFERENCES CITED

30. The following references are of record in the file of this patent:

#### UNITED STATES PATENTS

| Number    | Name         | Date          |
|-----------|--------------|---------------|
| 3,019,834 | Vierling     | Nov. 5, 1935  |
| 2,313,953 | Loughborough | Mar. 16, 1943 |
| 2,346,286 | Berliner     | Apr. 11, 1944 |
| 2,376,200 | Smidth       | May 15, 1945  |
| 2,398,649 | Kvalnes      | Apr. 16, 1946 |

#### OTHER REFERENCES

Stamm-Industrial & Eng. Chemistry, Oct. 1936, vol. 28, No. 10, pps. 1164-1169.

45. Pacific Plastics, vol. 2, No. 1, Jan. 1944, pps. 14 and 15.

Berliner Plastics (Chicago), July 1944, pps. 32-34, 90, 91.